

May 29, 1973

S. H. KAPLAN  
APERTURE MASK FOR, AND METHOD OF SCREENING, A COLOR  
CATHODE-RAY TUBE

3,736,137

Filed Oct. 22 1971

2 Sheets-Sheet 1



May 29, 1973

S. H. KAPLAN

3,736,137

APERTURE MASK FOR, AND METHOD OF SCREENING, A COLOR  
CATHODE-RAY TUBE

Filed Oct. 22 1971

2 Sheets-Sheet 2



FIG. 3

FIG. 4



FIG. 5

1

3,736,137

APERTURE MASK FOR, AND METHOD OF  
SCREENING, A COLOR CATHODE-RAY TUBE  
Sam H. Kaplan, Chicago, Ill., assignor to Zenith Radio  
Corporation, Chicago, Ill.  
Filed Oct. 22, 1971, Ser. No. 191,653  
Int. Cl. G03c 5/00

U.S. CL. 96—36.1

4 Claims

## ABSTRACT OF THE DISCLOSURE

The screen of a color cathode-ray tube is formed by means of a photographic method in which a photosensitive coating applied to the screen area is exposed through the apertures of a shadow mask. To obtain phosphor dots that are smaller in size than the apertures of the mask and larger in the center than at the edges of the screen, the mask apertures, which initially are of the same diameter, are temporarily closed down by the application of a removable coating having a thickness which increases progressively with radial spacing from the center toward the edge of the mask. After the screening is completed, the coating is removed from the apertures, conditioning the mask for utilization as the color selection electrode of the tube.

## BACKGROUND OF THE INVENTION

Methods for screening a shadow mask type of color cathode-ray tube are now quite well known and generally involve the use of a photosensitive coating to be exposed with the shadow mask in its operative relation relative to the screen to the end that the phosphor dots have the necessary precise position for color selection and color purity in the operation of the tube. The most popular screening technique is one in which the screen is covered with a photosensitive resist having the property that elemental areas which are exposed to actinic energy directed thereto through the apertures of the shadow mask become insoluble in a solvent. Conveniently, sensitized polyvinyl alcohol is used as a resist because it is soluble in water and, consequently, exposing this resist to develop an image of exposed dots permits easy development of that image simply by washing the screen with water. If the resist further includes a phosphor material as an ingredient, such an exposure and developing procedure permits the formation of the green phosphor dots, for example, of the screen. Repeating this same process twice more, suitably adjusting the position of the source of actinic energy on each occasion, results in depositing like dots of blue and red phosphor. Necessarily, the dot patterns are interlaced and collectively they define the now familiar mosaic or triad structure of the color screen.

It has become commonplace to arrange matters such that the phosphor dots of all three colors are of uniform size and larger in diameter than the electron beams which have access to the phosphor dots through the shadow mask. It has further become common practice to provide that the portion of the phosphor dots excited by an impinging electron beam be largest at the center of the screen and decrease in size with radial spacing from the center toward the edge of the screen or image area. This is accomplished by using a shadow mask in which the apertures are similarly graded in diameter with radial spacing from the center. An advantage, of course, is that a brightness increase is realized in the central portion of the screen and an acceptable tolerance for beam registration is made available at the edges of the screen where the possibility of misregistration is most pronounced. Screening with a mask of graded apertures in attempting to form dots of uniform size over the whole screen area has heretofore been difficult because of an undesired de-

2

pendence of the size of the phosphor dots upon the duration of the exposure step.

Another problem presents itself in constructing the screen for such a tube if it is to feature the so-called "black surround" principle described and claimed in Pat. 3,146,368, issued to Joseph P. Fiore et al., on Aug. 25, 1964, and assigned to the assignee of the present invention. This technique is one wherein both the brightness and contrast properties of a color tube are materially enhanced by having the phosphor dots smaller than the apertures of the shadow mask and by surrounding each such dot with light absorbing pigment. The practical difficulty here resides in attaining the desired relative dimensions of the phosphor dots and the apertures of the shadow mask. It has been proposed that the shadow mask have apertures of uniform diameter, temporarily stepped down by coating or plating with opaque material to the end that smaller diameter holes are available for screening purposes. After the screening, of course, the coating is removed so that the mask as permanently installed in the tube has larger apertures than the phosphor dots. Once again, the screening has been undesirably critical as to exposure time and also it has been a problem, heretofore, to conveniently attain a desired gradation of dots over the screen area in a tube having black surround and a shadow mask with apertures of uniform dimension. It is, therefore, an object of the invention to provide a novel aperture mask for, and method of screening, a color cathode-ray tube.

It is a particular object of the invention to provide a novel mask and screen for making color tube having black surround.

It is still a further object of the invention to provide a simplified and improved method of screening a color tube whether or not it features black surround.

## SUMMARY OF THE INVENTION

An aperture mask, in accordance with the invention, for a color cathode-ray tube has a pattern of apertures of predetermined relative diameter and further has a removable coating for the apertures which coating varies in thickness with the spacing of the apertures along radial directions from the center to the edge of the aperture pattern. For the conventional type of shadow mask tube the apertures of the mask, without the coating, are graded, increasing in diameter with radial distance and the coating thickness variation causes the apertures to have essentially uniform diameter for screening purposes.

On the other hand, the mask for a black surround type of shadow mask tube has apertures of substantially uniform diameter without the removable coating but in the presence of a coating of variable thickness the diameter decreases progressively with radial spacing from the center to the edge of the mask.

The method of the invention for screening a color cathode-ray tube having a black surround involves the presence of a coating of variable thickness the diameter of the apertures of the color selection electrode by applying thereto a removable coating having a thickness that varies with the spacing of the apertures along radial directions from the center to the edges of the aperture pattern. Having thus modified the diameters of the mask apertures or holes, a screen is formed on the faceplate comprising interleaved patterns of different phosphor materials individually applied by coating the faceplate with a photosensitive composition and exposing that coating with actinic energy through the coated mask to establish a latent image, and developing that image in an assigned one of the phosphor materials. After the screen has been formed the temporary coating of the color selection coating or mask is removed.

## BRIEF DESCRIPTION OF THE DRAWING

FIG. 1, is a schematic representation, in cross section, of a three-gun shadow mask color television tube screened in accordance with the method of the invention;

FIG. 2 is a simplified schematic view of a shadow mask embodying the invention and useful in screening the tube of FIG. 1;

FIG. 3 includes characteristic curves used in explaining the screening process;

FIG. 4 is a schematic view of another form of shadow mask in accordance with the invention; and,

FIG. 5 includes characteristic curves used in explaining screening practices to which the mask of FIG. 4 is relevant.

## DESCRIPTION OF THE PREFERRED EMBODIMENTS

The type of color television tube under consideration, as shown in FIG. 1, has an envelope 20 which conveniently has a faceplate section 21 dimensioned and configured for frit sealing to the conical section of the remainder of the envelope and the small end of the conical section terminates in the usual reduced diameter neck section. The faceplate section 21 is initially separate from the rest of the envelope which facilitates providing on the inner surface of the faceplate a screen 22 which is backed by a conductive and light reflecting layer 23. Screen 22 is comprised of a repeating series of phosphor triads each of which has a dot of green, a dot of blue and a dot of red phosphor all as well understood in the art and the backing layer 23 is usually formed of aluminum. A color selection electrode 24 or shadow mask is mounted contiguous to and in spaced parallel relation relative to the screen, being retained in position by mounting springs which connect at one end to the mask structure and terminate at the opposite ends in apertures dimensioned to receive support pins which project inwardly of the faceplate section of the tube envelope. This mounting arrangement is well known in the art, and, accordingly, has not been illustrated.

The neck portion of the envelope accommodates an arrangement of three electron guns 25, 26 and 27 which usually are assembled into what is referred to as a gun mount for issuing three electron beams designated R, B and G which are admitted to screen 22 by the apertures of the shadow mask 24. Since this is a parallax type of device, the geometry of the gun mount is such that the beam issuing from any of the three guns is permitted to see and impact upon only those phosphor dots of the color to which that particular beam has been assigned. There is one aperture of the shadow mask for each triad or dot cluster on the screen and the three beams scan the screen through the shadow mask under the influence of deflection fields generated by a deflection yoke 28. It has also been found necessary to provide a convergence field by means of a convergence assembly 29 so that the three beams maintain a desired condition of convergence in the plate of the shadow mask as these beams are deflected through the scanning raster.

The structure as thus far described is entirely conventional both as to its makeup and operation so that it is not necessary to consider such matters further and particular attention will be given to changes in the shadow mask and in the methods of screening.

Initial consideration will be given to forming a screen for a black surround tube. There are two approaches available; (1) applying the black surround material first and following this with the application of the interleaved patterns of phosphor dots, or (2) first establishing the interleaved patterns of dots of different phosphor materials followed by the application of black surround material. Both procedures are discussed in Pat. 3,146,368. Another and particularly attractive method of applying the black surround material first is described and claimed in an application of Sam H. Kaplan, Ser. No. 773,830, filed Nov. 75

6, 1968, and assigned to the assignee of the present invention. In view of these disclosures, and especially that of the afore-identified patent, it is not necessary to consider all of the manipulative steps of forming the screen; it is sufficient to consider the apparatus and process changes of the present invention.

Consider initially a previous process in which the shadow mask is formed with apertures of essentially uniform diameter but which are temporarily stepped down or reduced in size by a removable coating of a metal or an opaque organic material. For example, the mask may be plated with copper or zinc to provide the apertures with a temporary lining or coating that may be finally selectively removed by etching. Let it also be assumed that this lining or coating is of uniform thickness as proposed heretofore. To form one series of phosphor dots with such a shadow mask, the inner surface of the faceplate is coated with a photosensitive composition which usually is polyvinyl alcohol sensitized with ammonium dichromate but also, of course, including particles of the phosphor material from which the phosphor dots are desired to be formed. The faceplate having received a uniform coating of the photosensitive material is exposed with actinic energy, such as ultraviolet light, through shadow mask 24 to establish a latent image of the phosphor dot pattern in the coating which is easily developed in the phosphor being processed simply by washing with water after the exposure has taken place. As stated above, the elemental areas of the coating that have been exposed become insoluble whereas the unexposed portions retain their solubility in water and, therefore wash off leaving the exposed phosphor dots. FIG. 3 includes a curve A which shows the dependence of the size or dimension of the phosphor dot with exposure where exposure is the product of the intensity of the ultraviolet light and time or the exposure interval. This, of course, assumes exposure through an aperture of fixed dimension and with a light of a given or particular intensity. It is clear from curve A that the dot attains a maximum size after exposure for a certain minimum time which is apparent from the fact that the curve attains essentially zero slope after exposure  $e_1$ . In screening as conducted in the past, the point  $a_1$  of curve A represents the exposure conditions at the center of the screen resulting in a dot dimension in that portion of the screen of a diameter  $d_1$ . At the same time, conditions at the edge of the screen are represented at the point  $a_2$  of the curve which establishes a smaller dot size  $d_2$  at the edges of the screen or image area of the tube. This change in size is accomplished by changing the intensity of the exposure at these points of the screen since the duration of exposure is the same for both. Control of the intensity of the exposing light is made possible by the interposition of a graded light filter between the source and the shadow mask. The filter permits a desired gradation of phosphor dots from a maximum dimension at the center to the minimum dimension at the edges of the screen. But the criticalness of screening is apparent in considering the conditions at the point  $a_2$ . This falls at a steeply sloped part of the curve and, therefore, the dot size is subject to substantial variations with such things as exposure time and intensity, humidity, coating thickness and the like which is undesirable.

This limitation of prior practices is avoided by the present invention in accordance with which the thickness of the removable coating of the mask apertures varies with spacing of the apertures along radial directions from the center to the edge of the aperture pattern. Preferably, and as schematically illustrated in FIG. 2, the coating  $c_1$  at the center of the mask is less than the coating  $c_2$  spaced radially from the center. The coating increases progressively with increasing radial spacing of the apertures. For such a coated mask with resulting graded apertures or holes, the exposure conditions are represented by curve B in addition to curve A of FIG. 3. Curve B, while of the

same general shape as curve A, is for exposure through apertures at the edge of the mask which are smaller, in the face of removable coating  $c_2$ , than the apertures at the center of the mask and, therefore, give rise to smaller size dots for otherwise equal or equivalent conditions of exposure. In practicing the invention, the thickness variations of the removable coatings of the mask holes is such that exposure through the holes at the center of the mask result in maximum dot size  $d_1$  and exposure at the edge of the mask likewise gives maximum but a smaller dot size  $d_2$ . A family of similar curves, located between curves A and B could be drawn to show the equivalent conditions established at the intermediate apertures between the center and the edges of the mask. The advantage is apparent that the dot size is now essentially independent of exposure time because the exposure interval is at least that which results in maximum dot size and the condition represented at point  $a_2$  of curve A no longer prevails.

A 23 inch 90 degree shadow mask tube may be processed, in accordance with the invention, with an aperture mask having holes with a uniform diameter of about 16 mils. Such a mask is differentially coated to change the effective hole diameter from a value of 10.5 mils at the center decreasing progressively to about 7.5 mils at the edges. If the faceplate is coated with the conventional sensitized PVA slurry of uniform thickness and the exposure interval is sufficient that dot sizes of maximum dimension are attained, as described above, there will result a desired condition of graded dots varying in dimension from approximately 13 mils at the center to 10 mils at the edge of the screen. After the screening has been completed, including the usual filming and aluminizing, the removable coating is eliminated to restore the mask to its original condition in which it exhibits holes of uniform diameter. The tube now has maximum brightness at the center because of a larger dot size at that portion of the screen and also has desirable tolerance with respect to beam landings at the edge of the screen because of the reduced dot size at that portion of the screen.

It is not especially difficult to differentially coat the apertures of a shadow mask. Generally, plating is performed by immersing the mask in a suitable coating bath, using the mask as one electrode and having a cooperating and generally similarly shaped electrode in spaced relation with respect to the mask. If the other electrode is shaped so that its spacing from the mask is a minimum at the edges and a maximum at the center, the desired differential coating will result. In particular, the coating will be thicker at the edges and progressively thinner at apertures displaced radially inwardly toward the center of the mask.

Another advantage of the described process for the black surround type of screen is that it also grades the dots as explained, with the larger dots at the center for increased brightness.

The advantage of the described process in having the dot size less critically dependent on exposure conditions is also applicable to color tubes that do not employ black surround. Such a tube, as currently fabricated, uses a shadow mask in which the holes are graded, progressively decreasing in diameter from approximately 12 mils at the center to about 9½ mils at the edges. When employing such a mask in photographic type of screening, the exposure conditions are similar to those represented by curves F and G of FIG. 5. Curve F depicts conditions at the center of the screen above where the exposure is through the largest holes of the mask and curve G represents the other extreme, namely, conditions at the edge where the exposure is through holes of the mask having the smallest diameter. The operating points designated  $f_1$  and  $g_1$  are chosen to the end that the phosphor dots have essentially the same diameter over the screen. But here again, the operating point  $f_1$  is clearly

undesirably subject to variations in the parameters of the screening and exposure.

The modified mask shown in schematic form in FIG. 4 overcomes this difficulty through the technique of differential coating. In this case, the coating thickness increases from the edge of the pattern of apertures in the mask toward the center and at such a rate that the coated mask has holes of essentially uniform diameter since essentially uniform diameter dots are now required. The appropriate relation of dot size to exposure for the coated mask, for which the holes are not only uniform but are slightly smaller than the minimum dimension of the graded mask, is that of curve H and now the operating point is designated  $h$ . Operating at that point provides the same size phosphor dots as obtained from the aforescribed operation at the points  $f_1$  and  $g_1$  but now the dot size is much less dependent on precision of the exposure conditions since point  $h$  is on the flat part of the characteristic curve H.

In coating the graded screen, in the manner represented in FIG. 4, the coating thickness may be chosen to establish an overall hole diameter of about 9 mils and the exposure time and intensity may be adjusted to achieve the desired dot size  $d_3$  of approximately 17 mils.

While particular embodiments of the invention have been shown and described, it will be obvious to those skilled in the art that changes and modifications may be made without departing from the invention in its broader aspects, and, therefore, the aim in the appended claims is to cover all such changes and modifications as fall within the true spirit and scope of the invention.

I claim:

1. The method of screening a color cathode-ray tube of the type that has a color-selection electrode provided with a pattern of apertures for admitting electrons to a screen on the faceplate of said tube which method comprises:

modifying the diameter dimension of said apertures of said color-selection electrode by applying thereto a removable coating of opaque material having a thickness that varies with the spacing of said apertures along radial directions from the center to the edge of said aperture pattern;

forming a screen on said faceplate having interleaved patterns of different phosphor materials individually applied by (a) coating said faceplate with a photo-sensitive composition which becomes insoluble in a given solvent upon exposure to actinic energy, (b) exposing said photosensitive coating with actinic energy through said coated color-selection electrode to establish a latent image in said photosensitive coating comprised of insolubilized elemental areas that have been exposed and (c) developing said image in an assigned one of said phosphor materials by treating said screen with said solvent to remove all portions of said composition that remain unexposed;

and removing said coating of opaque material from said color-selection electrode after said screen has been formed.

2. The method in accordance with claim 1 in which: said latent image comprises a series of dots corresponding in number to the number of apertures in said color-selection electrode,

in which said photosensitive composition has the property that an image dot attains a maximum size upon exposure for a given time interval, and in which the relative diameters of said coated apertures establish said dots of said image at a predetermined relative size in response to exposure to actinic energy for at least said given time interval.

3. The method in accordance with claim 2 in which: said color-selection electrode, without said removable coating, has apertures of substantially uniform diameter,

in which said coating thickness increases progressively with the radial spacing of said apertures from the center of said electrode.

4. The method in accordance with claim 2 in which the apertures of said color-selection electrode, in the absence of said removable coating, have a diameter dimension that decreases with radial spacing from the center of said electrode,

an in which said removable coating causes the diameter dimension of said apertures to be substantially uniform.

10

## References Cited

## UNITED STATES PATENTS

|             |        |         |       |         |
|-------------|--------|---------|-------|---------|
| 3,645,734   | 2/1972 | Noguchi | ----- | 96—36.1 |
| 3,231,380   | 1/1966 | Law     | ----- | 96—36.1 |
| 5 2,755,402 | 7/1956 | Morrell | ----- | 96—36.1 |

NORMAN G. TORCHIN, Primary Examiner

R. L. SCHILLING, Assistant Examiner

U.S. Cl. X.R.

313—86, 92 B, 92 CS